

July 9, 1946.

R. L. HARVEY

2,403,657

INSULATING AND DIELECTRIC MATERIALS

Filed Jan. 29, 1943



Robert L. Harvey

Inventor

C. L. Harvey

Attorney

Patented July 9, 1946

2,403,657

# UNITED STATES PATENT OFFICE

2,403,657

## INSULATING AND DIELECTRIC MATERIAL

Robert L. Harvey, Princeton, N. J., assignor to  
Radio Corporation of America, a corporation  
of Delaware

Application January 29, 1943, Serial No. 473,937

1 Claim. (CL 260—41)

1

My present invention relates to insulating and dielectric materials for radio currents and has for its general object to provide an improved insulating and dielectric material having certain unique properties which render it especially suitable for use in electrical apparatus of the type designed to handle currents of ultra-high-frequencies, including so-called "centimeter waves."

My invention will be described in connection with the accompanying drawing wherein the single figure comprises a group of comparative curves showing how the  $Q$

$$\left( \frac{Q \text{ reactance}}{\text{resistance}} \right)$$

of certain materials changes with frequency.

It is known to those skilled in the art to which my invention appertains that the  $Q$  of the usual insulating materials, including the common thermo-plastic and thermo-setting resins, decreases with an increase in frequency. Thus, as shown by the curve which is designated "A" in the accompanying chart, polystyrene (or "styro," as it is sometimes called) exhibits a  $Q$  which decreases from a high value of approximately 6,000 at frequencies of the order of 1 megacycle to a value of less than 2,000 when subjected to frequencies in the 600-1,000 megacycle range.

It is also known that if two dielectric materials, such, for example, as polystyrene and silica dioxide (see curve "B"), are mixed together, the resulting compound will possess a  $Q$  lower than either of its constituents at any given frequency and, like its separate constituents, will exhibit a decrease in  $Q$  with an increase in frequency.

There are numerous applications in radio and analogous communication systems of the type utilizing ultra-high-frequencies for an insulating or dielectric material which will exhibit a constant  $Q$  or a rising  $Q$ , with an increase in frequency. By way of example; in a transmission line wherein losses normally increase with frequency due to redistribution of the current (i. e., "skin effect") a material having a  $Q$  which increases with frequency could be employed as dielectric and/or insulating material to compensate for such losses. A material which exhibits a flat  $Q$  or a rising  $Q$ , with an increase in frequency can also be used to advantage, either alone or in combination with other materials, as the dielectric medium in electric capacitors of various types and ratings. By way of example, such capacitors could be used in installations wherein it is desired to vary the selectivity of the

tuned circuits in a desired manner, with frequency.

Accordingly, a specific object of my invention is to provide an improved insulating and dielectric material for currents of radio frequencies, and one which shall exhibit a flat "Q" or, alternatively, a rising "Q" with an increase in frequency, and this, too, at frequencies of upwards of five million cycles (5 megacycles) per second.

Another and important object of my present invention is to achieve the aforesaid highly desirable and unique characteristics in a material having satisfactory heat resisting properties.

The foregoing and other objects are achieved in accordance with my invention by the addition, to moldable types of insulating compounds, prior to the molding operation, of a metal of low specific resistance, such for example, as copper or silver, in a finely divided state. The specific resistance of copper is  $1.7 \times 10^{-8}$ ; that of silver is  $1.6 \times 10^{-8}$ .

In carrying my invention into effect I prefer to employ polystyrene as the basic insulating ingredient because of its relatively high "Q" value, though I may employ other thermoplastic or thermosetting insulating materials, such for example as the phenol aldehyde, urea aldehyde and furfural resins, and to use copper particles of, say, 300 mesh as the metallic filler. The mixing may be carried out with the insulating material either in the powder or liquid form.

As shown by curve C of the drawing, the addition of substantially 10% by weight of copper particles to polystyrene results in a moldable non-conductive compound which exhibits a substantially constant  $Q$  over a frequency range of from, say, 5 to 400 megacycles. In order to achieve a  $Q$  which increases with frequency I employ a greater percentage of powdered metal. Thus, referring to curve D, I have found that the addition of 35% by weight of powdered copper to polystyrene results in a compound which exhibits a uniformly rising  $Q$  in the 5 to 400 megacycle band. Curves E and F show that over the same frequency range a somewhat lower  $Q$ , but one which nevertheless increases with frequency, is achieved when the percentage of copper in the compound is increased to 50% and 70% respectively.

I have found that the addition of the powdered metal to the conventional insulating materials increases the usable temperature range of such materials. Thus, in the case of polystyrene the usable temperature range is increased from 75° C. to, say, 90° C.

As a result of my work with these dielectric

3

compounds over a wide frequency range I have reason to believe that the slope of the curves C, D, E and F remain substantially the same as indicated in the drawing at frequencies of the order of several thousand megacycles, but owing to the possibility of error in making the necessary measurements at these frequencies with present day apparatus and technique, I have omitted such representation from the drawing.

I claim:

An electrical insulating and dielectric medium

4

consisting of polystyrene and distributed throughout a finely divided metal selected from the group consisting of copper and silver in the proportion of from 10 percent to 35 percent by weight of the polystyrene, said medium exhibiting a ratio of reactance to resistance within the frequency range of from 5 megacycles per second to 1,000 megacycles per second which has a value at least as great at the higher of said frequencies as at the lower of said frequencies.

ROBERT L. HARVEY.